

2,994,662

## LUBRICATING COMPOSITIONS

George M. Calhoun, Berkeley, and William A. Hewett, Oakland, Calif., assignors to Shell Oil Company, a corporation of Delaware

No Drawing. Filed Dec. 2, 1957, Ser. No. 699,919  
18 Claims. (Cl. 252—48.6)

This invention relates to lubricants, particularly those useful for lubrication under severe operating conditions, such as under extreme high speed and at high temperatures.

It is well known that the high pressure occurring in certain types of gears and bearings may cause rupture of lubricant films with consequent damage to the machinery. It is known that various base lubricants can be improved in their protective properties for rubbing surfaces by the addition of certain substances, so-called extreme pressure agents, so that excessive wear, scuffing and seizure which normally follow a break in the film lubricant are minimized or prevented.

It is known that certain compounds of metal-reactive elements, such as certain compounds of chlorine, sulfur and phosphorus, as well as certain other compounds, such as some compounds of lead, impart extreme pressure properties to various lubricants. Notable among the substances heretofore used are the lead soaps, phosphoric acid esters, free or bound sulfur and certain chlorinated organic compounds. A principal objection to many of these extreme pressure agents is their generally high reactivity with the metallic surface, causing etching, corrosion and discoloration of the metal surface. Another objection to chemically reactive extreme pressure agents is that they alter the original chemical nature of the contacting surface, which under certain conditions is undesirable. Additionally, because of the activity of agents of this type, they usually are depleted rapidly resulting in only a temporary solution to the problem of extreme pressure lubrication.

It has now been discovered that improved extreme pressure lubricants are provided by a suitable lubricating oil containing certain essentially oil-soluble sulfur-containing carboxylic acids having the formula



wherein R is an oil-solubilizing hydrocarbyl radical, preferably a  $\text{C}_8$ — $\text{C}_{30}$  alkyl radical, R' is hydrogen or a short alkyl radical of from 1 to 4 carbon atoms, Y is an oxygen-containing radical such as  $-\text{COOX}$ ,  $-\text{OH}$ , etc., preferably  $-\text{COOH}$  or  $-\text{OH}$ , X is hydrogen or a hydrocarbyl radical, m is an integer of at least 7 and n is an integer of from 1 to 4, preferably 1, and at least one of the Y groups or  $-\text{COOR}'$  carboalkoxy being a carboxylic acid or carboxy ( $-\text{COOH}$ ) radical.

Compounds of the type represented by the above formula can be prepared by reacting a mercapto acid or ester with an unsaturated acid or other equivalent compound. The mercapto acid or ester has the formula

$\text{HSR}''-\text{COOR}'$

wherein R'' is an alkylene radical of not more than 4 carbon atoms, e.g. mercaptoacetic acid, alpha- and beta-mercaptopropionic acid, alpha-, beta- and gamma-mercaptopropionic acid and O-mercaptopvaleric acid, methyl or ethyl mercapto-acetate, propionate or butyrate. The unsaturated long-chain acidic compound may be a long-chain unsaturated fatty acid, e.g. oleic acid, linoleic acid, linolenic acid, erucic acid, ricinoleic acid or an unsaturated fatty alcohol, e.g. oleyl alcohol, ricinoleyl alcohol, etc. Instead of the free acids or alcohols these com-

pounds can be used in the form of their esters, e.g. methyl or ethyl oleate, lauryl oleate, glycerol trioleate or the like.

The additives used in oil compositions of this invention can be prepared by the methods described by Koenig et al., JACS 79, 362 (1957), or Fitzgerald, Jr., Org. Chem. 22, 197 (1957), or by any other suitable means and preferably at low temperatures (from room temperature to about 50° C.) and in the presence of a free radical catalyst such as azo or peroxide catalysts or ultra-violet light and a non-reactive solvent such as benzene, toluene, xylene, or the like. Suitable initiators include various free radical-yielding initiators, for example, various organic peroxides, such as aliphatic, aromatic, heterocyclic and alicyclic peroxides, such as diethyl peroxide, tertiary butyl hydroperoxide, dibenzoyl peroxide, diterbutyl peroxide, dimethylthienyl peroxide, dicyclohexyl peroxide, dilauroyl peroxide and urea peroxide. These are mentioned by way of non-limiting examples of suitable organic peroxides. Other initiating compounds known include emulsion redox systems, such as a mixture of sodium bisulfite and persulfate, ammonium persulfate, alkali metal perborates, azo compounds, such as alpha, alpha-azodiisobutyronitrile, etc.

The following examples illustrate the preparation of suitable additives for use in oil compositions in accordance with the present invention.

### EXAMPLE I

About 600 grams of oleic acid and 223.5 grams of mercapto-acetic acid were mixed in a flask at 20—25° C. About 240 drops (30 drops at a time) of t-butyl hydroperoxide were added over a period of 2 hours and the temperature was kept at about 37° C. The reaction mixture was diluted with 2 volumes of diethyl ether, washed with 12 liters of water to pH 4, dried over  $\text{Na}_2\text{SO}_4$ , filtered and the solvent stripped at 155° C. and 2 mm. pressure. The final product was a mixture of 9- and 10-carboxymethylmercaptopstearic acid and analysis of the product was as follows:

|             | Percent<br>C | Percent<br>H | Percent<br>O | Percent<br>S | Eq. Wt. |
|-------------|--------------|--------------|--------------|--------------|---------|
| Found.....  | 64.2         | 10.2         | 17.0         | 8.74         | 183     |
| Theory..... | 64.2         | 10.23        | 17.10        | 8.56         | 187     |

### EXAMPLE II

About 600 grams of ethyl oleate and 223.5 grams of mercaptoacetic acid were mixed in a flask at 20—25° C. About 240 (30 drops at a time) of t-butyl hydroperoxide were added over a period of 2 hours and the temperature was kept at about 37° C. The reaction mixture was diluted with 2 volumes of diethyl ether, washed with 12 liters of water to pH 4, dried over  $\text{Na}_2\text{SO}_4$ , filtered and the solvent stripped at 155° C. and 2 mm. pressure. The final product was a mixture of ethyl 9- and 10-carboxymethylmercaptopstearate and analysis of the product was as follows:

|             | Percent<br>C | Percent<br>H | Percent<br>O | Percent<br>S | Eq. Wt. |
|-------------|--------------|--------------|--------------|--------------|---------|
| Found.....  | 65.7         | 10.5         | 16.0         | 7.75         | 472     |
| Theory..... | 65.6         | 10.51        | 15.9         | 7.96         | 402     |

### EXAMPLE III

About 600 grams of ricinoleic acid and 223.5 grams of mercaptoacetic acid were mixed in a flask at 20—25° C. About 240 drops (30 drops at a time) of t-butyl hydroperoxide were added over a period of 2 hours and the temperature was kept at about 27° C. The reaction mixture was diluted with 2 volumes of diethyl ether, washed

with 12 liters of water to pH 4, dried over  $\text{Na}_2\text{SO}_4$ , filtered and the solvent stripped at 155° C. and 2 mm. pressure. The final product was a mixture of 9- and 10-carboxymethylmercapto-12-hydroxystearic acid and the equivalent weight of the product was found to be 207 (theory 195).

#### EXAMPLE IV

About 600 grams of glyceryl trioleate and 223.5 grams of mercaptoacetic acid were mixed in a flask at 20-25° C. About 240 drops (30 drops at a time) of t-butyl hydroperoxide were added over a period of 2 hours and the temperature was kept at about 37° C. The reaction mixture was diluted with 2 volumes of diethyl ether, washed with 12 liters of water to pH 4, dried over  $\text{Na}_2\text{SO}_4$ , filtered and the solvent stripped at 155° C. and 2 mm. pressure. The final product was a mixture of glyceryl tris(9- and 10-carboxymethylmercaptooleate) and the equivalent weight of the product was found to be 445 (theory 387).

#### EXAMPLE V

About 600 grams of oleyl alcohol and 223.5 grams of mercaptoacetic acid were mixed in a flask at 20-25° C. About 240 drops (30 drops at a time) of t-butyl hydroperoxide were added over a period of 2 hours and the temperature was kept at about 37° C. The reaction mixture was diluted with 2 volumes of diethyl ether, washed with 12 liters of water to pH 4, dried over  $\text{Na}_2\text{SO}_4$ , filtered and the solvent stripped at 155° C. and 2 mm. pressure. The final product was a mixture of 9- and 10-carboxymethylmercaptooleate alcohol.

The mercapto-modified acids or alcohols in general are oil-soluble and can be used in amounts of from about 0.5% to about 20%, preferably from about 1% to about 5% by weight. Although these mercapto-modified acids or alcohols are oil-soluble some of them form opaque solutions which can be overcome and the solutions rendered transparent by addition to oils containing these mercapto products a small amount (0.1-10%) of an oil-soluble branched-chain aliphatic monohydric alcohol, oil-soluble high molecular weight fatty acid or monoester of said fatty acid and polyhydric alcohols. The alcohols, fatty acids or monoesters can effectively clarify oils containing mercapto acids or alcohols or derivatives thereof as described without destroying the extreme pressure properties of such oil compositions.

The oil-soluble alkanols particularly useful as clarifiers are the so-called "Oxo" alcohols derived from branched-chain olefins, such as polymers of lower alkenes of 3 to 5 carbon atoms, and copolymers of mixtures of such alkenes, by catalyzed reaction with carbon monoxide and hydrogen in accordance with the conditions of the "Oxo" process, as is well known in the art. The composition of a typical  $\text{C}_8$ -Oxo-alcohol mixture derived from a mixture of  $\text{C}_7$ -olefins, produced by polymerization of a typical refinery cracked gas fraction of  $\text{C}_3$ - $\text{C}_4$  hydrocarbons is given in Table I.

Table I

| Alcohol              | Percent, wt. |
|----------------------|--------------|
| 3,5-dimethyl hexanol | 29           |
| 4,5-dimethyl hexanol | 25           |
| 3,4-dimethyl hexanol | 17           |
| 5-methyl heptanol    | 1.4          |
| 3-methyl heptanol    | 1.4          |
| 5-ethyl hexanol      | 2.3          |
| 5,6-dimethyl hexanol | 4.3          |
| alpha-alkyl alkanols | 4.3          |
| Others               | 5.0          |

Other examples of suitable alkanols include 6-methyl-1-heptanol, 2-n-propyl-1-pentanol, 3-n-propyl-1-hexanol, 2,2-dimethyl-1-octanol, 10,10-dimethyl-1-undecanol, 3-isopropyl-1-heptanol and mixtures thereof.

The fatty acids useful as clarifiers include the saturated and unsaturated oil-soluble fatty acids having from 10

to 30 carbon atoms such as capric, lauric, oleic, linoleic, ricinoleic acids and mixtures thereof.

The monoesters derived from simple alkane polyols and long chain fatty acids useful as clarifiers include 5 oil-soluble glycerol monooleate, glycerol monostearate, glycerol monoricinoleate, pentaerythritol mono- and di-laureate, pentaerythritol mono- and dioleate, pentaerythritol mono- and distearate, mono-, di-, and triethylene glycol monooleate, propylene glycol monoricinoleate, triethylene glycol monostearate, sorbitol monolaurate, mannositol monooleate, mannositol dioleate, sorbitol dioleate, etc.

The lubricating oils used in compositions of this invention can be a variety of synthetic or natural hydrocarbon oils having a viscosity range of from 50 SUS at 100° F. to 250 SUS at 210° F. (SAE viscosity number ranging from SAE 5 to SAE 90). The natural hydrocarbon oils can be obtained from paraffinic, naphthenic, asphaltic or mixed base crudes, and/or mixtures thereof. Synthetic oils include polymerized olefins, alkylated aromatics, isomerized waxes, copolymers of alkylene glycols and alkylene oxide (Ucon fluids) which are described in U.S. Patents 2,425,755, 2,425,845 and 2,774,733 such as Ucon 50HB170, Ucon 50HB660 or Ucon LB550X and which are copolymers of ethylene and 1,2-propylene oxides the mono and diols as well as their ether derivatives; organic esters of an aliphatic dibasic acid such as di-2-ethyl hexyl sebacate or di-2-ethyl hexyl adipate and the like. The hydrocarbon oils may be blended with fixed oils such as castor oil, lard oil and the like and/or synthetic oils as mentioned or silicone polymers and the like. Typical oils of this type are petroleum motor oils (A) which is paraffinic in character and (B) which is naphthenic in character having the following properties:

|                               | (A) (SAE 10W) | (B) (SAE 30) |
|-------------------------------|---------------|--------------|
| Pour Point, ° F.....          | -10           | -5           |
| Flash, ° F.....               | 300           | 415          |
| Viscosity, SUS at 210° F..... | 44            | 58           |
| Viscosity Index.....          | 90            | 60           |

Other suitable oils are the gas turbine lube oils having the following properties:

|                               | Grade..... | 1010 | 1065 |
|-------------------------------|------------|------|------|
| Flash, COC, ° F.....          | 300        | 465  |      |
| Pour, ° F.....                | -10        | 0    |      |
| Viscosity, SUS at 100° F..... | 59.4       | 530  |      |
| Neutral Number.....           | 0.02       | 0.01 |      |
| Ash.....                      | None       | None |      |

The following compositions are illustrative of the invention; the percentages being by weight.

|    |                                                                    |         |
|----|--------------------------------------------------------------------|---------|
| 55 | Composition A:                                                     | Percent |
|    | Example I additive.....                                            | 2       |
|    | 1010 mineral oil.....                                              | Balance |
| 60 | Composition B:                                                     |         |
|    | Example I additive.....                                            | 2       |
|    | Glycerol monooleate.....                                           | 2       |
|    | 1010 mineral oil.....                                              | Balance |
| 65 | Composition C:                                                     |         |
|    | Example III additive.....                                          | 2       |
|    | Glycerol monooleate.....                                           | 8       |
|    | 1010 mineral oil.....                                              | Balance |
| 70 | Composition D:                                                     |         |
|    | Example IV additive.....                                           | 2       |
|    | Glycerol monooleate.....                                           | 5       |
|    | 1010 mineral oil.....                                              | Balance |
| 75 | Composition E:                                                     |         |
|    | Example II additive.....                                           | 2       |
|    | 1010 mineral oil.....                                              | Balance |
| 80 | Composition F:                                                     |         |
|    | Example V additive.....                                            | 2       |
|    | $\text{C}_{13}\text{H}_{27}\text{OH}$ (made by "Oxo" process)..... | 3.5     |
|    | 1010 mineral oil.....                                              | Balance |

## Composition G:

|                    |         |
|--------------------|---------|
| Example I additive | 2       |
| Lauric acid        | 2       |
| SAE 90 mineral oil | Balance |

## Composition H:

|                                          |         |
|------------------------------------------|---------|
| Example I additive                       | 2       |
| $C_{13}H_{27}OH$ (made by "Oxo" process) | 2.74    |
| SAE 90 mineral oil                       | Balance |

## Composition I:

|                                                                             |         |
|-----------------------------------------------------------------------------|---------|
| Example I additive                                                          | 5       |
| Ucon 50HB660 (polyethylene-propylene glycol having a SUS at 100° F. of 660) | 10      |
| Di-2-ethylhexyl sebacate                                                    | Balance |

## Composition J:

|                          |    |
|--------------------------|----|
| Example I additive       | 2  |
| Di-2-ethylhexyl sebacate | 15 |

Compositions of this invention were evaluated for their extreme pressure properties on a Spur-Gear machine. The machine consists essentially of two geometrically similar pairs of gears connected by two parallel shafts. The gear pairs are placed in separate gear boxes, which also contain the supporting ball bearings. One of the shafts consists of two sections connected by a coupling. Loading is accomplished by locking one side of the coupling and applying torque to the other. The conditions of the test were:

Speed r.p.m. 3200 and 10,000  
 Oil temperature °F. 100  
 Oil flow-rate cc./sec. 10  
 Load in increments 5 min. at each setting.

Results of the evaluations are given in Table I. For purpose of comparison, the results obtained from the use of the base oil alone, and with other dicarboxylic acids, are also given in Table II.

Table II

| Compositions                                             | Score Load, lbs./in.   |
|----------------------------------------------------------|------------------------|
| A                                                        | 12,700 (3,200 r.p.m.). |
| B                                                        | 9,900 (10,000 r.p.m.). |
| C                                                        | 9,900 (10,000 r.p.m.). |
| D                                                        | 9,900 (10,000 r.p.m.). |
| E                                                        | 7,800 (3,200 r.p.m.).  |
| F                                                        | 12,000 (3,200 r.p.m.). |
| 1010 Mineral oil+2% $C_{16}$ alkenyl succinic acid       | 1,400 (3,200 r.p.m.).  |
| 1010 Mineral oil+2% malonic acid                         | 2,800 (3,200 r.p.m.).  |
| 1010 Mineral oil+2% 3-hexadecyl adipic acid              | 1,400 (3,200 r.p.m.).  |
| 1010 Mineral oil+2% thiodiglycolic acid                  | 5,000 (3,200 r.p.m.).  |
| 1010 Mineral oil+2% thio alpha, alpha'-bis(stearic acid) | 3,500 (3,200 r.p.m.).  |
| 1010 Mineral oil+2% dodecyl-mercaptosuccinic acid        | 1,400 (10,000 r.p.m.). |
| 1010 Mineral oil+2% heptylmercaptosuccinic acid          | 4,200 (3,200 r.p.m.).  |
| 1010 Mineral oil+2% alpha-mercaptopbenzoic acid          | 4,200 (3,200 r.p.m.).  |
| 1010 Mineral oil+10% glycerol monooleate                 | 1,800 (3,200 r.p.m.).  |
| 1010 Mineral oil+13.25% lauric acid                      | 3,400 (3,200 r.p.m.).  |
| 1010 Mineral oil+2% $C_{13}H_{27}OH$ ("Oxo" process)     | 600 (3,200 r.p.m.).    |
| 1010 Mineral oil                                         | 600 (3,200 r.p.m.).    |

The data show the outstanding enhancement of the load-carrying ability of the oil effected by the mercapto-containing acids of the invention, as represented by those of Compositions A through F. On the other hand, malonic acid, succinic acid, 3-hexadecyl adipic acid and  $C_{16}$  alkenyl succinic acid as well as sulfur-containing acid outside the scope used by applicants such as thiodiglycolic acid, thio-alpha, alpha'-bis(stearic acid), dodecyl-mercaptosuccinic acid, heptylmercaptosuccinic acid, alpha-mercaptopbenzoic acid, glycerolmonooleate, lauric acid or "Oxo" alcohol effected only a slight improvement.

The sulfur-containing acids of this invention are useful also for providing superior load-carrying properties in lubricating oils which contain minor amounts of other agents which are non-reactive with the dicarboxylic acids, such as silicone anti-foaming agents, alkylphenol anti-oxidants, polyacrylate ester viscosity-index improvers, and the like.

We claim as our invention:

1. A lubricating oil composition comprising a major

amount of mineral lubricating oil and from about 1% to 5% of a sulfur-containing carboxylic acid having the formula



wherein R is an oil-solubilizing alkyl radical having from 8 to 30 carbon atoms, R' is selected from the group consisting of hydrogen and a  $C_1-C_4$  alkyl radical, Y is an oxygen-containing radical selected from the group consisting of  $-\text{OH}$  and  $\text{COOX}$  where X is selected from the group consisting of hydrogen and a hydrocarbyl radical, m is an integer of from 7 to 10 and n is an integer of from 1 to 4, one of the oxygen-containing groups being a carboxy radical.

2. A mineral lubricating oil composition comprising a major amount of mineral lubricating oil and from about 1% to 5% of a carboxy  $C_{1-4}$  alkyl mercapto-substituted long chain fatty acid, said carboxy  $C_{1-4}$  alkyl mercapto radical being from 7 to 10 carbon atoms away from the carboxyl radical of the fatty acid.

3. A mineral lubricating oil composition comprising a major amount of mineral lubricating oil and from about 1% to 5% of a carboxy  $C_{1-4}$  alkyl mercapto-substituted long chain fatty alcohol, said carboxy  $C_{1-4}$  alkyl mercapto radical being from 7 to 10 carbon atoms away from the hydroxyl radical of the fatty alcohol.

4. A mineral lubricating oil composition comprising a major amount of mineral lubricating oil and from about 1% to 5% of a carboxy  $C_{1-4}$  alkyl mercapto-substituted ester of a long chain fatty acid, said carboxy  $C_{1-4}$  alkyl mercapto radical being from 7 to 10 carbon atoms away from the ester group.

5. A mineral lubricating oil composition comprising a major amount of mineral lubrication oil and from about 1% to 5% of a carboxy methyl mercapto-substituted long chain fatty acid, said methyl mercapto radical being from 7 to 10 carbon atoms away from the carboxyl radical of the fatty acid.

6. The lubricating oil composition of claim 1 containing from about 0.1% to about 10% of an oil-soluble monoester of a fatty acid having 10-30 carbon atoms and a glycerol.

7. The lubricating oil composition of a claim 1 containing from about 0.1% to about 10% of an oil-soluble branched-chain Oxo alcohol.

8. The lubricating oil composition of claim 1 containing from about 0.1% to about 10% of an oil-soluble long-chain fatty acid having 10-30 carbon atoms.

9. A mineral lubricating oil composition comprising a major amount of mineral lubricating oil and from about 1% to 5% of 9- and 10-carboxymethylmercaptopstearic acid.

10. A mineral lubricating oil composition comprising a major amount of mineral lubricating oil and from about 1% to about 5% of 9- and 10-carboxymethylmercaptop-2-hydroxystearic acid.

11. A mineral lubricating oil composition comprising a major amount of mineral lubricating oil and from about 1% to about 5% of glycerol tris(9- and 10-carboxymethylmercaptopstearate).

12. A mineral lubricating oil composition comprising a major amount of mineral lubricating oil and from about 1% to about 5% of ethyl 9- and 10-carboxymethylmercaptopstearate.

13. A mineral lubricating oil composition comprising a major amount of mineral lubricating oil and from about 1% to about 5% of 9- and 10-carboxymethylmercaptopstearyl alcohol.

14. The lubricating oil composition of claim 9 containing from about 0.1% to about 10% of glycerol monooleate.

15. The lubricating oil composition of claim 9 containing from about 0.1% to about 10% of lauric acid.

16. The lubricating oil composition of claim 9 con-

taining from about 0.1% to about 10% of an oil-soluble branched-chain Oxo alcohol.

17. The lubricating oil composition of claim 9 containing from about 0.1% to about 10% of glycerol monooleate.

18. The lubricating composition of claim 12 containing from about 0.1% to about 10% of an oil-soluble branched-chain Oxo alcohol.

5

References Cited in the file of this patent

UNITED STATES PATENTS

|           |                |                |
|-----------|----------------|----------------|
| 2,317,666 | Burwell et al. | Apr. 27, 1943  |
| 2,449,996 | Gresham et al. | Sept. 28, 1948 |
| 2,459,717 | Perry          | Jan. 18, 1949  |
| 2,644,793 | Rudel et al.   | July 7, 1953   |
| 2,737,525 | Mulvaney       | Mar. 6, 1956   |